

Nov. 19, 1929.

H. J. BLUHM

1,736,425

BOWLING PIN

Filed Feb. 16, 1925

Fig. 1



Fig. 2



Inventor:

Harold J. Bluham

By: *J. A. Reel*  
Atty.

## UNITED STATES PATENT OFFICE

HAROLD J. BLUHM, OF MUSKEGON HEIGHTS, MICHIGAN, ASSIGNOR TO THE BRUNSWICK-BALKE-COLLENDER COMPANY, OF WILMINGTON, DELAWARE, A CORPORATION OF DELAWARE

## BOWLING PIN

Application filed February 16, 1925. Serial No. 9,515.

This invention relates to bowling pins, and has for its object to provide a durable and substantial bowling pin which can be made to conform to standard regulations as to size, shape and weight, which will not crack, split or splinter in actual use, and which will give a good sound when struck by a bowling ball or by other pins.

Further objects are to provide a pin which will have a smooth surface and an attractive appearance, which will not chip or wear off quickly at the base, which will not break easily at the neck, which can be made at comparatively low cost, and which will give better service than all-wood pins and be more satisfactory to players.

My invention relates to pins made of a plastic composition in the form of a shell or as a covering for a core of any suitable construction and material and its object is to provide a plastic composition which will produce a stronger and more substantial bowling pin than has been customary with plastic compositions heretofore used for that purpose.

It is understood, of course, that my improved plastic composition can be utilized in making bowling pins of many varieties as to structure. I have selected one simple form of shell and an improved form of that shell, to illustrate my invention, but without limiting the invention to these particular structures.

In the accompanying drawing,

Fig. 1 shows a bowling pin in the form of a hollow shell.

Fig. 2 also shows a bowling pin in the form of a hollow shell with a neck relatively softer than the body and the head.

I have found it satisfactory to provide a plastic composition consisting of a hard rubber compound for stock of which the pin is made, and I add fiber to the compound to increase the strength of the pin. I have found that cotton fiber and sisal fiber may be satisfactorily used, but I prefer the cotton fiber because it gives better results, and I may use any fiber equivalent or substantially equivalent to cotton fiber or sisal fiber, which will give satisfactory results.

The addition of the fiber to the compound

provides a stock which produces a bowling pin having greater strength than plastic composition pins heretofore made. The fiber constitutes a finely divided and widely distributed reinforcing and strengthening binder which increases the strength of the pin and likewise increases its resistance to the blows and rough usage to which bowling pins are subjected, and which might otherwise result in injury to the pin.

My invention may be embodied in a shell of the simple form shown in Fig. 1 or of the form shown in Fig. 2, wherein the neck 3 is softer than the body 4 and head 5, as more fully set forth in my companion application filed concurrently herewith. The shell may be provided with a core of any suitable material and construction or the shell itself may have reinforcements molded thereon, and it will be understood that I do not limit the invention to use with shells of any particular kind, but desire to cover it broadly for the manufacture of bowling pins of any kind, shape and construction, within the scope of the following claims.

I claim:

1. A bowling pin having a hard body portion and a flexible neck portion said neck portion being made of a rubber composition and reinforced by fibre incorporated therein.

2. A bowling pin having a body portion made of hard rubber composition and a neck portion made of relatively soft rubber composition both of said portions being reinforced by fibre incorporated therein.

3. A shell-like bowling pin having a hollow interior and comprising a body portion made of a relatively hard rubber composition and a neck portion made of a relatively soft rubber composition, both of said portions being reinforced by fibre incorporated therein.

HAROLD J. BLUHM.